# EUROPEAN PATENT SPECIFICATION

(11) **EP 3 748 079 B1**
(45) Date of publication and mention of the grant of the patent: **31.05.2023**
(21) Application number: 19746956.2
(22) Date of filing: 22.01.2019
(51) Int. Cl.: D21H 27/10, A24D 1/02, A24D 1/04

(54) **PACKING MATERIAL FOR COUPLING MULTIPLE SEGMENTS CONSTITUTING SMOKING PRODUCT**
VERPACKUNGSMATERIAL ZUR KOPPLUNG VON MEHREREN SEGMENTEN EINES RAUCHARTIKELS
MATÉRIAU D'EMBALLAGE POUR L'ACCOUPLEMENT DE MULTIPLES SEGMENTS CONSTITUANT UN PRODUIT À FUMER

(30) Priority: 01.02.2018 KR 20180013065
(43) Date of publication of application: 09.12.2020
(73) Proprietor: KT&G Corporation, Daedeok-gu Daejeon 34337 (KR)
(72) Inventor: CHEONG, Bong Su, Daejeon 34128 (KR); LEE, John Tae, Daejeon 34118 (KR); HWANG, Jung Seop, Daejeon 34071 (KR); JIN, Yong Sook, Daejeon 34885 (KR); KI, Sung Jong, Daejeon 34127 (KR)
(74) Representative: Ter Meer Steinmeister & Partner
(86) International application number: PCT/KR2019/000871
(87) International publication number: WO 2019/151695

(56) References cited:
- WO-A1-2016/156219
- WO-A1-2017/041920
- JP-A- 2000 064 192
- KR-A- 910 001 175
- KR-A- 20080 111 521
- KR-A- 20100 093 285

## Description

### TECHNICAL FIELD

The present disclosure relates to a packing material that combines a plurality of segments constituting a smoking article.

### BACKGROUND ART

In recent years, there has been an increasing demand for alternative methods of overcoming the shortcomings of general smoking articles. For example, there is an increasing demand for a method of generating an aerosol by heating an aerosol-generating material in a smoking article rather than a method of burning a smoking article to produce an aerosol. Accordingly, research into a heating-type smoking article or a heating-type aerosol-generating apparatus has been actively conducted.

The existing combustion-type smoking articles are generally composed of a smoking material section and a filter section. Referring to an existing combustion-type smoking article 10 shown in FIG. 1, a cylindrical first rod section is formed as a smoking material section 100 is wrapped by a first cover 100a, and a cylindrical second rod section is formed as a filter section (i.e., a plurality of filters 110 and 120) is wrapped by one or more second covers 110a, 120a, and 130. The first rod section and the second rod section are coupled to each other by a tip paper 140 wrapping a portion of the first rod section and the entire second rod section.

The length of the smoking material section 100 in the existing combustion-type smoking article 10 is generally about 57 mm, and the length of the filter section including the plurality of filters 110 and 120 is about 27 mm. In general, a region where a user bites the smoking article 10 when smoking is located about 12 mm from the end of the filter section, and thus, when the filter portion includes the plurality of filters 110 and 120, the region where a user bites the smoking article 10 when smoking may correspond to a position where the plurality of filters 110 and 120 abut each other. However, even if the region where a user bites the smoking article 10 when smoking corresponds to the position where the plurality of filters 110 and 120 abut each other, a portion corresponding to the plurality of filters 110 and 120 may not be broken because the tip paper 140 surrounds the plurality of filters 110 and 120 as a whole.

As described above, the tip paper 140 has an advantage of preventing the filter section including the filters 110 and 120 from being broken. However, in order to manufacture the smoking article 10 including the tip paper 140, three or more layers of paper materials (i.e., the second covers 110a, 120a, and 130 and the tip paper 140) have to be provided, and thus, the manufacturing process of the smoking article 10 is complicated and the cost of the smoking article 10 is high. Accordingly, there is a need for a technology that simplifies the manufacturing process of a smoking article and reduces the manufacturing cost thereof.
WO 2016/156219 A1 relates to an electrically heated aerosol-generating article comprising an aerosol-generating substrate, a mouthpiece, and a paper wrapper circumscribing at least a portion of the aerosol-generating substrate. The aerosol-generating substrate comprises at least one aerosol former in an amount of between about 5 percent and about 30 percent by weight of the aerosol-generating substrate. The paper wrapper has a wet tensile strength of at least about 5 Newtons per 15 mm when measured in accordance with the Wet Tensile Strength Test.

### DESCRIPTION OF EMBODIMENTS

### SOLUTION TO PROBLEM

A packing material combining a plurality of segments constituting a smoking article may have a basis weight of 60 gsm or more and a tensile strength of 6.0 kgf/15 mm or more, and the average length of cellulose pulp fibers constituting the packing material may be in a range of 1.5 mm or more and 2.5 mm or less.

### ADVANTAGEOUS EFFECTS OF DISCLOSURE

The present disclosure may provide a packing material that combines a plurality of segments constituting a smoking article. Specifically, the packing material according to the present disclosure may have a basis weight of 60 gsm or more and a tensile strength of 6.0 kgf/15 mm or more, and the average length of cellulose pulp fibers constituting the packing material may be in a range of 1.5 mm or more and 2.5 mm or less.

Because the packing material according to the present disclosure has a high basis weight and a high tensile strength by adjusting the average length of cellulose pulp fibers constituting the packing material, even if the smoking article does not include a separate tip paper, a plurality of segments in the smoking article may be stably combined. Accordingly, the manufacturing process of the smoking article may be simplified, and the manufacturing cost of the smoking article may be reduced.

### BRIEF DESCRIPTION OF DRAWINGS

FIG. 1 is a view showing an example of a combustion-type smoking article according to the related art;
FIG. 2 is a view showing an example of a smoking article according to some embodiments;
FIG. 3 is a view showing a scanning electron microscope (SEM) image of cellulose pulp fibers constituting a packing material according to some embodiments; and
FIG. 4 is a view showing another example of a smoking article according to some embodiments.

### BEST MODE

A packing material combining a plurality of segments constituting a smoking article may have a basis weight of 60 gsm or more and a tensile strength of 6.0 kgf/15 mm or more, and the average length of cellulose pulp fibers constituting the packing material may be in a range of 1.5 mm or more and 2.5 mm or less.

The packing material may have a basis weight of 60 gsm or more and 100 gsm or less, and the average length of the cellulose pulp fibers constituting the packing material may be in a range of 1.8 mm or more and 2.1 mm or less.

The plurality of segments may include, in order, a smoking material section, an intermediate structure, a cooling structure, and a filter, and the packing material may be formed to entirely wrap the plurality of segments.

The smoking material section, the intermediate structure, the cooling structure, and the filter may be wrapped by separate covers, respectively, and the packing material may be formed to entirely wrap the smoking material section, the intermediate structure, the cooling structure, and the filter, which are wrapped by the separate covers, respectively.

The plurality of segments may include, in order, a front filter, a smoking material section, an intermediate structure, and a rear filter, and the packing material may be formed to entirely wrap the plurality of segments.

The front filter, the smoking material section, the intermediate structure, and the rear filter may be wrapped by separate covers, respectively, and the packing material may be formed to entirely wrap the front filter, the smoking material section, the intermediate structure, and the rear filter, which are wrapped by the separate covers, respectively.

### MODE OF DISCLOSURE

Hereinafter, embodiments shown only as examples will be described in detail with reference to the accompanying drawings. Descriptions will be given below for only specifying the embodiments and will not limit or restrict the scope of claims of the disclosure.

It will be further understood that the terms "comprises," "comprising," "includes" and/or "including," when used herein, do not necessarily indicate all of stated features, integers, steps, operations, elements, and/or components described in the specification and may preclude some of the stated features, the integers, steps, operations, elements, and/or components. Also, the terms do not preclude the presence or addition of one or more other features, integers, steps, operations, elements, components, and/or groups thereof.

Also, it will be understood that, although the terms first, second, etc. may be used herein to describe various elements, these elements should not be limited by these terms. These terms are only used to distinguish one element from another.

The terms used in the disclosure are selected from among common terms that are currently widely used in consideration of their function in the disclosure. However, the terms may be different according to an intention of one of ordinary skill in the art, a precedent, or the advent of new technology. Also, in particular cases, the terms are discretionally selected by the applicant of the disclosure, and the meaning of those terms will be described in detail in the corresponding part of the detailed description. Therefore, the terms used in the disclosure are not merely designations of the terms, but the terms are defined based on the meaning of the terms and content throughout the disclosure.

The present embodiments relate to a packing material that combines a plurality of segments constituting a smoking article. Aspects well known to one of ordinary skill in the art will not be described in detail.

FIG. 2 is a view showing an example of a smoking article according to some embodiments.

Referring to FIG. 2, a smoking article 20 may include a smoking material section 210, an intermediate structure 220, a cooling structure 230, a filter 240, a first cover 210a, a second cover 220a, a third cover 230a, a fourth cover 240a, and a packing material 250. The smoking article 20 may be a heating-type cigarette used with an aerosol-generating apparatus.

The smoking material section 210 may contain an aerosol-generating material. For example, the smoking material section 210 may include a strand of tobacco.

For example, the aerosol-generating material may include at least one of glycerin, propylene glycol, ethylene glycol, dipropylene glycol, diethylene glycol, triethylene glycol, tetraethylene glycol, and oleyl alcohol.

The smoking material section 210 may have an elongated rod shape, and the length of the smoking material section 210 may vary and may, in an optional embodiment, be about 7 millimeters to about 15 millimeters, for example, 12 millimeters. Furthermore, the diameter of the smoking material section 210 may be about 7 millimeters to about 9 millimeters, for example, 7.9 millimeters.

In an alternative embodiment, the smoking material section 210 may contain other additives such as a flavoring agent, a wetting agent and/or an acetate compound. For example, the flavoring agent may include licorice, sucrose, fructose syrup, isosweet, cocoa, lavender, cinnamon, cardamom, celery, fenugreek, cascarilla, sandalwood, bergamot, geranium, honey essence, rose oil, vanilla, lemon oil, orange oil, mint oil, cinnamon, caraway, cognac, jasmine, chamomile, menthol, ylang-ylang, salvia, spearmint, ginger, coriander, coffee, or the like. In addition, the wetting agent may include glycerin, propylene glycol, or the like.

In an alternative embodiment, the smoking material section 210 may include a reconstituted tobacco material having a piece such as a rod. The reconstituted tobacco material may be prepared by grinding a tobacco raw material, mixing a solvent and various additives in the ground tobacco raw material to make a slurry-like material, drying the slurry-like material to form a sheet, and then processing the sheet.

For example, the smoking material section 210 may include a plurality of strands of tobacco material. One strand may have a length of about 10 millimeters to about 14 millimeters (e.g., 12 millimeters), a width of about 0.8 millimeters to about 1.2 millimeters (e.g., 1 millimeter), and a thickness of about 0.08 millimeters to about 0.12 millimeters (e.g., 0.1 millimeters).

By allowing the smoking material section 210 to include a plurality of stranded materials obtained by processing a wide tobacco sheet form, aerosol generation may increase as the density of a tobacco material filled in the smoking material section 210 increases, and manufacturing characteristics of the smoking material section 210 may be improved.

The filter 240 may be arranged in a direction facing the smoking material section 210 and may be an area through which an aerosol material generated in the smoking material section 210 passes immediately before a user inhales the aerosol material.

The filter 240 may include various materials, for example, cellulose acetate.

In an alternative embodiment, the filter 240 may include a recess filter including a hollow.

In an alternative embodiment, the length of the filter 240 may be about 5 millimeters to about 15 millimeters.

In an alternative embodiment, the filter 240 may include at least one capsule (not shown). The capsule (not shown) provided in the filter 240 may have a structure in which a content liquid containing a fragrance is wrapped with a film, and may have, for example, a spherical or cylindrical shape.

In addition, a material forming the film of the capsule (not shown) provided in the filter 240 may be starch and/or a gelling agent. For example, gellan gum or gelatin may be used as the gelling agent. Furthermore, a gelling aid may be further used as the material forming the film of the capsule (not shown). In this case, for example, calcium chloride may be used as the gelling aid. Furthermore, a plasticizer may be further used as the material forming the film of the capsule (not shown). In this case, glycerin and/or sorbitol may be used as the plasticizer. In addition, a coloring agent may be further used as the material forming the film of the capsule (not shown).

For example, menthol, essential oil of a plant, etc. may be used as the fragrance contained in the content liquid of the capsule. In addition, for example, a medium-chain triglyceride (MCT) may be used as a solvent of the fragrance contained in the content liquid. In addition, the content liquid may contain other additives such as a pigment, an emulsifier, and a thickener.

The intermediate structure 220 may be arranged between the filter 240 and the smoking material section 210, for example, adjacent to the smoking material section 210.

The intermediate structure 220 may include various materials, for example, may include cellulose acetate.

In an alternative embodiment, the intermediate structure 220 may be in the form of a tube including a hollow formed therein.

The length of the intermediate structure 220 may be about 7 millimeters to about 15 millimeters, for example, 7 millimeters. In addition, the length of the intermediate structure 220 may be variously set, and the entire length of the smoking article 20 may be controlled according to the length of the intermediate structure 220.

The cooling structure 230 may be arranged between the smoking material section 210 and the filter 240, specifically, between the intermediate structure 220 and the filter 240. In an alternative embodiment, the cooling structure 230 may contact the intermediate structure 220 and the filter 240.

The cooling structure 230 may cool an aerosol generated in the smoking material section 210. This allows a user to inhale an aerosol at an appropriate and safe temperature that is not too high.

For example, when the smoking article 20 is inserted into an aerosol-generating apparatus and used, the cooling structure 230 may cool an aerosol generated as a heater provided in the aerosol-generating apparatus heats the smoking material section 210.

The length of the cooling structure 230 may be about 10 millimeters to about 20 millimeters, for example, 14 millimeters.

The cooling structure 230 may include various materials. For example, the cooling structure 230 may contain poly lactic acid (PLA).

The cooling structure 230 may be manufactured in various ways. In an alternative embodiment, the cooling structure 230 may be manufactured (e.g., woven) using fibers containing poly lactic acid, in which case the risk that the cooling structure 230 is deformed or loses function by an external impact may be lowered. In addition, by changing a method of combining the fibers, a cooling structure 230 having various shapes may be manufactured.

In addition, by manufacturing the cooling structure 230 by using fibers, a surface area in contact with the aerosol may increase. Therefore, an aerosol cooling effect of the cooling structure 230 may be further improved.

The first cover 210a may be formed to wrap the smoking material section 210, and the second cover 220a may be formed to wrap the intermediate structure 220. Each of the first cover 210a and the second cover 220a may include various materials, for example, papers. In an alternative embodiment, each of the first cover 210a and the second cover 220a may include papers having oil resistance.

The third cover 230a may be formed to wrap the cooling structure 230, and the fourth cover 240a may be formed to wrap the filter 240. Each of the third cover 230a and the fourth cover 240a may include various materials, for example, general papers (including hard paper).

In an alternative embodiment, each of the third cover 230a and the fourth cover 240a may include papers having oil resistance.

The packing material 250 may be formed to entirely wrap a plurality of segments constituting the smoking article 20. For example, the packing material 250 may be formed to entirely wrap the smoking material section 210, the intermediate structure 220, the cooling structure 230, and the filter 240. In addition, the packing material 250 may contact the first cover 210a, the second cover 220a, the third cover 230a, and the fourth cover 240a while wrapping the first cover 210a, the second cover 220a, the third cover 230a, and the fourth cover 240a.

When the basis weight of the packing material 250 increases, the tensile strength of the packing material 250 also increases. In addition, when the basis weight and tensile strength of the packing material 250 increases, the stiffness of the packing material 250 increases, and thus, as the basis weight and tensile strength of the packing material 250 increases, the plurality of segments wrapped by the packing material 250 may be stably combined, and when a user smokes, the possibility that the smoking article 20 composed of the plurality of segments is broken may be lowered.

However, when the basis weight and tensile strength of the packing material 250 excessively increases, it may be difficult to manufacture the smoking article 20 as a cylindrical rod due to resilience caused by the high stiffness of the packing material 250. Therefore, it is necessary to determine the ranges of basis weight and tensile strength at which the plurality of segments wrapped by the packing material 250 may be stably combined and the smoking article 20 may be easily manufactured as a rod.

Table 1 below is a table showing the degree of breakage of the smoking article 20 in a border region between the plurality of segments according to the basis weight and tensile strength of the packing material 250. In Table 1, the degree of breakage of the smoking article 20 in the border region between the plurality of segments was determined by a sensory evaluation based on the number of broken smoking articles when 20 smoking articles 20 were smoked.

**[Table 1]**

| | | | | |
|---|---|---|---|---|
| basis weight (g/m²) | 40 | 60 | 80 | 100 |
| tensile strength (kgf/15mm) | 4.7 | 6.3 | 9.0 | 11.1 |
| degree of breakage in border region between plurality of segments | 14 (insufficient) | 1 (good) | 0 (good) | 0 (good) |

Referring to Table 1, when the basis weight of the packing material 250 is 60 gsm or more and the tensile strength of the packing material 250 is 6.3 kgf/15 mm or more, the degree of breakage in the border region between the plurality of segments is 1 or less, and thus, it can be seen that the packing material 250 has sufficient stiffness (corresponding to good). Therefore, the packing material 250 may be manufactured to have a basis weight of 60 gsm or more and a tensile strength of 6.0 kgf/15 mm or more.

Table 2 below is a table summarizing how many minutes a rod manufacturing operation is performed under the condition that a combiner speed is 500 rod per minute (rpm), in order to determine whether it is easy to manufacture the smoking article 20 as a rod (it is assumed that the circumference of the rod is 23 mm.).

**[Table 2]**

| | | | | | |
|---|---|---|---|---|---|
| basis weight (g/m²) | 30 | 60 | 80 | 100 | 115 |
| stiffness (cm³) | 15 | 50 | 100 | 150 | 200 |
| rod manufacturing operation time (500 rpm, up to 10 minutes operation) | 10 minutes operation | 10 minutes operation | 10 minutes operation | 1 minute operation | inoperability (jam occurs due to bursting of packing material) |
| rod manufacturing workability | good | good | good | insufficient | bad |

Referring to Table 2, it can be seen that when the basis weight of the packing material 250 exceeds 100 gsm, the stiffness of the packing material 250 excessively increases, resulting in insufficient rod manufacturing workability. Therefore, the basis weight of the packing material 250 has to be determined to be 100 gsm or less in order to be easy enough to manufacture the smoking article 20 as a rod. Therefore, the packing material 250 may be manufactured to have a basis weight of 60 gsm or more and 100 gsm or less.

The tensile strength of the packing material 250 is closely related to the lengths of cellulose pulp fibers constituting the packing material 250. For example, Table 3 below is a table showing the tensile strength of packing material 250 according to the average length of cellulose pulp fibers constituting the packing material 250 when the basis weight of packing material 250 is 60 g/m².

**[Table 3]**

| | | | |
|---|---|---|---|
| average length of cellulose pulp fibers (mm) | 2.1 | 2.0 | 1.8 |
| tensile strength (kgf/15mm) | 7.5 | 8.3 | 8.5 |
| freeness (SR) | 20 | 25 | 33 |

Referring to Table 3, it can be seen that the tensile strength of the packing material 250 increases as the average length of the cellulose pulp fibers constituting the packing material 250 decreases. Specifically, by increasing the freeness, a combination area between the cellulose pulp fibers constituting the packing material 250 may increase, and as the freeness increases, the cellulose pulp fibers are softened and fibrillated to improve contact between the cellulose pulp fibers. Therefore, the tensile strength of the packing material 250 may increase. In addition, as the tensile strength of the packing material 250 increases, the stiffness of the packing material 250 may also increase. Therefore, it can be seen that adjusting the average length of the cellulose pulp fibers constituting the packing material 250 may determine the basis weight or tensile strength of the packing material 250 in an appropriate range.

According to the results of the experiment, the average length of the cellulose pulp fibers constituting the packing material 250 has to be determined in a range of 1.5 mm or more and 2.5 mm or less in order for the packing material 250 to have a basis weight of 60 gsm or more and 100 gsm or less and a tensile strength of 6.0 kgf/15 mm or more. For example, the average length of the cellulose pulp fibers constituting the packing material 250 may be determined in a range of 1.8 mm or more and 2.1 mm or less. Hereinafter, the cellulose pulp fibers constituting the packing material 250 will be described in more detail with reference to FIG. 3.

FIG. 3 is a view showing a scanning electron microscope (SEM) image of cellulose pulp fibers constituting a packing material according to some embodiments.

Referring to FIG. 3, it can be seen that the packing material 250 is formed by combining a plurality of cellulose pulp fibers with each other. When the average length of the plurality of cellulose pulp fibers is reduced, the tensile strength of the packing material 250 including the plurality of cellulose pulp fibers may increase because a combination area between the plurality of cellulose pulp fibers increases.

The average length of the plurality of cellulose pulp fibers may be adjusted in order for the packing material 250 to have an appropriate range of tensile strength. For example, the average length of the plurality of cellulose pulp fibers may be determined in a range of 1.5 mm or more and 2.5 mm or less. In this case, that the average length of the plurality of cellulose pulp fibers is in a range of 1.5 mm or more and 2.5 mm or less may mean that the length of any cellulose pulp fiber 30 among the plurality of cellulose pulp fibers is 1.5 mm or more and 2.5 mm or less.

FIG. 4 is a view showing another example of a smoking article according to some embodiments.

Referring to FIG. 4, a smoking article 40 may include a front filter 410, a smoking material section 420, an intermediate structure 430, a rear filter 440, a first cover 410a, a second cover 420a, a third cover 430a, a fourth cover 440a, and a packing material 450. Description that is the same as that given with reference to FIG. 2 may be omitted. The smoking article 40 may be a heating-type cigarette used with an aerosol-generating apparatus.

The smoking material section 420 may contain an aerosol-generating material. For example, the smoking material section 210 may include a strand of tobacco, or may include a tobacco material in the form of granules. However, the disclosure is not limited thereto.

The front filter 410 and the rear filter 440 may be arranged at both ends of the smoking article 40, respectively, and may be areas through which an aerosol material generated in the smoking material section 420 passes. The front filter 410 and the rear filter 440 may include various materials. For example, the front filter 410 and the rear filter 440 may include cellulose acetate.

The intermediate structure 430 may be arranged between the rear filter 440 and the smoking material section 420, for example, adjacent to the smoking material section 420. The intermediate structure 430 may include various materials, for example, may include cellulose acetate.

The first cover 410a may be formed to wrap the front filter 410, and the second cover 420a may be formed to wrap the smoking material section 420. In addition, the third cover 430a may be formed to wrap the intermediate structure 430, and the fourth cover 440a may be formed to wrap the rear filter 440. Each of the first cover 410a, the second cover 420a, the third cover 430a, and the fourth cover 440a may include various materials, for example, papers. In an alternative embodiment, each of the first cover 410a, the second cover 420a, the third cover 430a, and the fourth cover 440a may include papers having oil resistance.

The packing material 450 may be formed to entirely wrap a plurality of segments constituting the smoking article 40. For example, the packing material 450 may be formed to entirely wrap the front filter 410, the smoking material section 420, the intermediate structure 430, and the rear filter 440. In addition, the packing material 450 may contact the first cover 410a, the second cover 420a, the third cover 430a, and the fourth cover 440a while wrapping the first cover 410a, the second cover 420a, the third cover 430a, and the fourth cover 440a.

The packing material 450 may have a suitable range of basis weight and tensile strength so that the smoking article 40 is easily manufactured as a rod while a plurality of segments wrapped by the packing material 450 may be stably combined. For example, the packing material 450 may have a basis weight of 60 gsm or more and a tensile strength of 6.0 kgf/15 mm or more. In addition, the packing material 450 may have a basis weight of 60 gsm or more and 100 gsm or less.

The average length of a plurality of cellulose pulp fibers constituting the packing material 450 may be adjusted in order for the packing material 450 to have an appropriate range of basis weight or tensile strength. For example, the average length of the plurality of cellulose pulp fibers constituting the packing material 450 may be determined in a range of 1.5 mm or more and 2.5 mm or less. In this case, that the average length of the plurality of cellulose pulp fibers is in a range of 1.5 mm or more and 2.5 mm or less may mean that the length of any cellulose pulp fiber among the plurality of cellulose pulp fibers is 1.5 mm or more and 2.5 mm or less. The average length of the plurality of cellulose pulp fibers constituting the packing material 450 may be determined in a range of 1.8 mm or more and 2.1 mm or less.

Because the packing material 250 and 450 according to the embodiment of the present disclosure has a high basis weight and tensile strength as the average length of the cellulose pulp fibers constituting the packing material 250 and 450 is adjusted, the plurality of segments provided in the smoking article 20 and 40 may be stably combined even if the smoking article 20 and 40 does not have separate tip paper. Accordingly, the manufacturing process of the smoking article 20 and 40 may be simplified, and the manufacturing cost of the smoking article 20 and 40 may be reduced.

## Claims

1. A packing material (250, 450) for combining a plurality of segments for constituting a smoking article (20, 40),
wherein the packing material (250, 450) has a basis weight of 60 gsm or more and a tensile strength of 6.0 kgf /15 mm or more, and
an average length of cellulose pulp fibers (30) constituting the packing material (250, 450) is in a range of 1.5 mm or more and 2.5 mm or less.

2. The packing material of claim 1, wherein the packing material (250, 450) has a basis weight of 60 gsm or more and 100 gsm or less.

3. The packing material of claim 1, wherein the average length of the cellulose pulp fibers (30) constituting the packing material (250, 450) is in a range of 1.8 mm or more and 2.1 mm or less.

4. The packing material of claim 1, wherein the plurality of segments include, in order, a smoking material section (210, 420), an intermediate structure (220, 430), a cooling structure (230), and a filter (240, 440), and
the packing material (250, 450) is formed to entirely wrap the plurality of segments.

5. The packing material of claim 4, wherein the smoking material section (210, 420), the intermediate structure (220, 430), the cooling structure (230), and the filter (240, 440) are wrapped by separate covers, respectively, and
the packing material (250, 450) is formed to entirely wrap the smoking material section (210, 420), the intermediate structure (220, 430), the cooling structure (230), and the filter (240, 440), which are wrapped by the separate covers, respectively.

6. The packing material of claim 1, wherein the plurality of segments include, in order, a front filter (410), a smoking material section (420), an intermediate structure (430), and a rear filter (440), and
the packing material (250, 450) is formed to entirely wrap the plurality of segments.

7. The packing material of claim 6, wherein the front filter (410), the smoking material section (420), the intermediate structure (430), and the rear filter (440) are wrapped by separate covers, respectively, and
the packing material (250, 450) is formed to entirely wrap the front filter (410), the smoking material section (420), the intermediate structure (430), and the rear filter (440), which are wrapped by the separate covers, respectively.

8. The packing material of any one of the previous claims, wherein the packing material combines a plurality of segments constituting a smoking article (20, 40).

9. Smoking article (20, 40) comprising a plurality of segments, wherein the plurality of segments is combined by a packing material (250, 450) according to any one of the previous claims.

## Patentansprüche

1. Verpackungsmaterial (250, 450) zum Kombinieren mehrerer Segmente zum Bilden eines Raucherzeugnisses (20, 40),
wobei das Verpackungsmaterial (250, 450) ein Grundgewicht von 60 gsm oder größer und eine Zugfestigkeit von 6,0 kgf/15 mm [58,84 N/15 mm] oder größer aufweist, und
eine durchschnittliche Länge der Zellulosezellstofffasern (30), die das Verpackungsmaterial (250, 450) bilden, in einem Bereich von 1,5 mm oder größer und 2,5 mm oder kleiner liegt.

2. Verpackungsmaterial nach Anspruch 1, wobei das Verpackungsmaterial (250, 450) ein Grundgewicht von 60 gsm oder größer und 100 gsm oder kleiner aufweist.

3. Verpackungsmaterial nach Anspruch 1, wobei die durchschnittliche Länge der Zellulosezellstofffasern (30), die das Verpackungsmaterial (250, 450) bilden, in einem Bereich von 1,8 mm oder größer und 2,1 mm oder kleiner liegt.

4. Verpackungsmaterial nach Anspruch 1, wobei die mehreren Segmente in dieser Reihenfolge einen Rauchmaterialabschnitt (210, 420), eine Zwischenstruktur (220, 430), eine Kühlstruktur (230) und einen Filter (240, 440) enthalten, und
das Verpackungsmaterial (250, 450) derart gebildet ist, dass es die mehreren Segmente vollständig umhüllt.

5. Verpackungsmaterial nach Anspruch 4, wobei der Rauchmaterialabschnitt (210, 420), die Zwischenstruktur (220, 430), die Kühlstruktur (230) und der Filter (240, 440) jeweils durch getrennte Umhüllungen umhüllt sind, und
das Verpackungsmaterial (250, 450) derart gebildet ist, dass es den Rauchmaterialabschnitt (210, 420), die Zwischenstruktur (220, 430), die Kühlstruktur (230) und den Filter (240, 440), die jeweils durch die getrennten Umhüllungen umhüllt sind, vollständig umhüllt.

6. Verpackungsmaterial nach Anspruch 1, wobei die mehreren Segmente in dieser Reihenfolge einen vorderen Filter (410), einen Rauchmaterialabschnitt (420), eine Zwischenstruktur (430) und einen hinteren Filter (440) enthalten, und
das Verpackungsmaterial (250, 450) derart gebildet ist, dass es die mehreren Segmente vollständig umhüllt.

7. Verpackungsmaterial nach Anspruch 6, wobei der vordere Filter (410), der Rauchmaterialabschnitt (420), die Zwischenstruktur (430) und der hintere Filter (440) jeweils durch getrennte Umhüllungen umhüllt sind, und
das Verpackungsmaterial (250, 450) derart gebildet ist, dass es den vorderen Filter (410), den Rauchmaterialabschnitt (420), die Zwischenstruktur (430) und den hinteren Filter (440), die jeweils durch die getrennten Umhüllungen umhüllt sind, vollständig umhüllt.

8. Verpackungsmaterial nach einem der vorhergehenden Ansprüche, wobei das Verpackungsmaterial mehrere Segmente kombiniert, die ein Raucherzeugnis (20, 40) bilden.

9. Raucherzeugnis (20, 40), das mehrere Segmente umfasst, wobei die mehreren Segmente durch ein Verpackungsmaterial (250, 450) nach einem der vorhergehenden Ansprüche kombiniert sind.

## Revendications

1. Matériau d'emballage (250, 450) pour combiner une pluralité de segments pour constituer un article à fumer (20, 40),
dans lequel le matériau d'emballage (250, 450) a un grammage de 60 g/m² ou plus et une résistance à la traction de 6,0 kgf /15 mm ou plus, et
une longueur moyenne de fibres de pâte cellulosique (30) constituant le matériau d'emballage (250, 450) est dans une plage de 1,5 mm ou plus et 2,5 mm ou moins.

2. Matériau d'emballage selon la revendication 1, dans lequel le matériau d'emballage (250, 450) a un grammage de 60 g/m² ou plus et 100 g/m² ou moins.

3. Matériau d'emballage selon la revendication 1, dans lequel la longueur moyenne des fibres de pâte cellulosique (30) constituant le matériau d'emballage (250, 450) est dans une plage de 1,8 mm ou plus et 2,1 mm ou moins.

4. Matériau d'emballage selon la revendication 1, dans lequel les segments de la pluralité de segments incluent, dans l'ordre, une section de substance à fumer (210, 420), une structure intermédiaire (220, 430), une structure de refroidissement (230) et un filtre (240, 440), et
le matériau d'emballage (250, 450) est formé de manière à envelopper entièrement la pluralité de segments.

5. Matériau d'emballage selon la revendication 4, dans lequel la section de substance à fumer (210, 420), la structure intermédiaire (220, 430), la structure de refroidissement (230) et le filtre (240, 440) sont enveloppés par des éléments de recouvrement séparés, respectivement, et
le matériau d'emballage (250, 450) est formé de manière à envelopper entièrement la section de substance à fumer (210, 420), la structure intermédiaire (220, 430), la structure de refroidissement (230) et le filtre (240, 440), qui sont enveloppés par les éléments de recouvrement séparés, respectivement.

6. Matériau d'emballage selon la revendication 1, dans lequel les segments de la pluralité de segments incluent, dans l'ordre, un filtre avant (410), une section de substance à fumer (420), une structure intermédiaire (430) et un filtre arrière (440), et
le matériau d'emballage (250, 450) est formé de manière à envelopper entièrement la pluralité de segments.

7. Matériau d'emballage selon la revendication 6, dans lequel le filtre avant (10), la section de substance à fumer (420), la structure intermédiaire (430) et le filtre (440) sont enveloppés par des éléments de recouvrement séparés, respectivement, et
le matériau d'emballage (250, 450) est formé de manière à envelopper entièrement le filtre avant (410), la section de substance à fumer (420), la structure intermédiaire (430) et le filtre arrière (440), qui sont enveloppés par les éléments de recouvrement séparés, respectivement.

8. Matériau d'emballage selon l'une quelconque des revendications précédentes, dans lequel le matériau d'emballage combine une pluralité de segments constituant un article à fumer (20, 40).

9. Article à fumer (20, 40) comportant une pluralité de segments, dans lequel la pluralité de segments est combinée par un matériau d'emballage (250, 450) selon l'une quelconque des revendications précédentes.
